

Dec. 8, 1953

J. B. DUKE ET AL

2,661,842

CONCENTRATION OF PHOSPHATE ORES

Filed Aug. 3, 1950



INVENTORS.  
JAMES B. DUKE  
WESLEY M. HOUSTON

BY

Williams, Rich, Moran

ATTORNEYS

## UNITED STATES PATENT OFFICE

2,661,842

## CONCENTRATION OF PHOSPHATE ORES

James B. Duke, Medulla, and Wesley M. Houston,  
Lakeland, Fla., assignors to Attapulgus Minerals & Chemicals Corporation, a corporation of Maryland

Application August 3, 1950, Serial No. 177,374

4 Claims. (Cl. 209—166)

1

The present invention relates to the concentration of phosphate minerals from their ores, and may be regarded as an improvement upon the method covered by the patent to Arthur Crago 2,293,640, issued August 18, 1942, now owned by the assignee of the present application.

That Crago patent describes a method of concentrating phosphate minerals from their ores, which comprises (in the first step) subjecting the ore in an aqueous pulp to a concentrating operation with negative-ion reagents to separate a rougher concentrate of the phosphate values admixed with entrained silicious gangue; treating the said rougher phosphate concentrate (in the second step) with a mineral acid to remove the effect, on both the phosphate and silica particles, of the negative-ion reagents used in the production of said rougher concentrate; and then (in the third step) subjecting the thus acid-treated rougher concentrate in an aqueous pulp to a concentrating operation with a positive-ion reagent which is a selective collector for the gangue in said rougher phosphate concentrate to separate from it a collected material largely composed of the silicious gangue, thereby producing a final phosphate concentrate.

The general object of the present invention is to improve the method described in said Crago patent so as to reduce the plant equipment required, and to economize in the quantity of positive-ion reagent employed, while still obtaining from the ore a phosphate concentrate having a low insoluble content and containing most of the phosphate in the ore.

These objects are attained by the method of the present invention which will be understood from the following description, taken in connection with the accompanying drawing showing a simplified general flow-sheet of a typical plant practicing the said method. It will be understood that this flow-sheet merely contributes to an understanding of the invention, and that various modifications in the apparatus may be resorted to without departing from the spirit of the invention as defined in the claims hereto appended.

In the flow-sheet drawing the four steps of the improved method are separated by dash lines and are marked 1, 2, 3 and 4. The first step 1 results in obtaining from the phosphate ore feed, by the use of negative-ion reagents (as in the method of the Crago patent) a rougher phosphate concentrate. The second step 2 involves subjecting said rougher concentrate in an aqueous pulp to retarded froth-flotation treatment,

2

thereby removing as a part of the final product a froth-product having a low insoluble content, and a middling residue which contains most of the silicious gangue and a considerable proportion of the phosphate in the rougher phosphate concentrate. In the third step 3 of the method, said middling is treated with a mineral acid and rinsed to remove the effect of the negative-ion reagents on the particles in the middling. In the fourth and last step 4, the thus acid-treated middling is subjected to a concentrating operation with a positive-ion reagent which is a collector for the silicious gangue thereby removing from said middling and sending to waste most of the silicious gangue, and producing as the machine-discharge a high-grade phosphate concentrate (having a low insoluble content) which is added to the previously mentioned high-grade phosphate concentrate to form the final phosphate product containing most of the phosphate in the original ore.

Examples of negative-ion reagents which may be used in the first step of the method, and examples of positive-ion reagents which may be used in the fourth step of the method are mentioned in said Crago patent. The mineral acid employed in the third step is preferably sulfuric acid, but other mineral acids such as nitric acid, hydrochloric acid and hydrofluoric acid may be used. In practicing the concentrating operations of the first, second and fourth steps, flotation cells have been found to be particularly satisfactory, but other forms of apparatus may be employed.

The meaning of "retarded flotation" in the second step of the method illustrated in the flow-sheet drawing will now be particularly described. As illustrated, to the rougher phosphate concentrate (supplied by the first step of the method) is added acidulated flotation water having a low pH, say about 3.0. Instead, however, of using acidulated flotation water having a low pH, we have found that it is possible to obtain the same result by subjecting the rougher phosphate concentrate to agitation and scrubbing with ordinary (neutral) flotation water. After the rougher phosphate concentrate has been treated in either of the ways mentioned, it is fed in an aqueous pulp to flotation cells in which the pulp, owing to either of the previous treatments mentioned, is subjected to what has been called a "retarded-flotation" treatment, thereby producing a high-grade phosphate concentrate froth-product (having a low insoluble content) which is a substantial part of the final phosphate concentrate; and a machine discharge which contains

almost all of the silicious gangue and a part of the coarser phosphate particles in the rougher phosphate concentrate. This is the middling material which is rich in phosphate and is treated in the third and fourth steps of the method.

It has been found that the rougher phosphate concentrate may be subjected to retarded-flotation treatment (in the second step of the method) by subjecting it to froth-flotation treatment in flotation cells in which the level of the pulp is maintained so low that only the top portion of the froth-product is removed. This froth-product is a high grade phosphate concentrate (having a low insoluble content); and the machine discharge from these cells, containing almost all of the silicious gangue and a considerable part of the coarser phosphate in the rougher phosphate concentrate, is the middling treated in the third and fourth steps of the method.

It will be apparent, therefore, that the second step of the method results in obtaining, by the retarded-flotation treatment of the rougher phosphate concentrate, by treatments which restrain the normal floatability of the rougher phosphate concentrate, a cleaner concentrate containing very little silicious gangue, and a middling containing the remainder of the coarser phosphate and most of the gangue in the rougher phosphate concentrate. The method which is the present invention, therefore, does not require the acid-treating (in the third step) and the flotation treatment with positive-ion reagents (in the fourth step) of all of the rougher phosphate concentrate, but merely the treating (in the third and fourth steps) of a much less weight of material than is the case in the second and third steps of the method of the Crago patent. The advantageous result is that the method of the present invention requires the use of less acid (in the third step) and the use of less positive-ion reagents (in the fourth step) than in the method of the Crago patent. The economy thus achieved in the use of positive-ion reagents was surprising and unpredictable, because the amount of silicious material floated in the last step of applicants' method is obviously substantially the same as the amount of such material floated in the last step of the Crago method. Moreover, since less weight of material is treated in the third and fourth steps of the present method than in the second and third steps of the method of the Crago patent, the plant equipment required is reduced.

To contribute to a clear understanding of the method which is the present invention, examples based on tests will now be described.

In each of the examples hereinafter described, the flotation feeds were composed of -35 mesh deslimed particles of bone phosphate of lime (B. P. L.) and silica sand.

#### Example I

This example illustrates the use of weakly-acid flotation water in the second step of the method.

A -35 mesh deslimed phosphate ore feed was conditioned in an aqueous pulp for 2 minutes at 70% solids with 0.5 pound of caustic soda, 3.0 pounds of fuel oil, and 0.37 pound of tall oil, all in pounds per ton of dry feed. The conditioned feed was diluted with tap water to about 20% solids in a minerals separation laboratory air-flow flotation machine, agitated and aerated to produce a sand tailing in the machine-discharge

and a froth-product which was a rougher phosphate concentrate containing entrained sand particles.

The rougher phosphate concentrate was de-watered and repulped in the flotation machine at about 10% solids with water to which sufficient sulfuric acid had been added to produce a pH of 3, employing approximately 3.0 pounds of  $H_2SO_4$  per ton of original feed. The rougher concentrate was agitated briefly and then aerated and re-flotted in this acid water producing a retarded-flotation of a high-grade cleaner phosphate concentrate containing a minimum sand content and a phosphate-rich middling machine-discharge consisting of both phosphate and sand particles.

The said rich middling was agitated for about 3 minutes at approximately 50% solids with 0.75 pound of sulfuric acid per ton of original feed, and was then washed and rinsed free of acid and spent negative-ion reagents. The acid-treated and rinsed middling was repulped in a flotation machine, conditioned for about 15 seconds with .025 pound of "Armac T" (tallow amine acetate made by Armour & Company), 0.1 pound of kerosene and 0.02 pound of pine oil frother (all in pounds per ton of original feed), and then was aerated and a low-grade silicious froth-product was removed and sent to waste, leaving a high-grade phosphate concentrate in the machine-discharge which was combined with the high-grade phosphate concentrate produced by the second step. The metallurgical results of this test are recorded in the following table:

#### ROUGHER PHOSPHATE FLOTATION

| Products                                | Percent weight | Percent B. P. L. | Percent insol. | Percent B. P. L. recovery |
|-----------------------------------------|----------------|------------------|----------------|---------------------------|
| 1. Feed                                 | 100.0          | 26.8             | -----          | 100.0                     |
| 2. Rougher concentrate froth-product    | 36.5           | 70.0             | -----          | 95.3                      |
| 3. Silicious machine-discharge to waste | 63.5           | 2.0              | -----          | 4.7                       |

#### RETARDED CLEANER FLOTATION

|                                        |      |      |       |      |
|----------------------------------------|------|------|-------|------|
| 4. Phosphate concentrate froth-product | 22.6 | 77.2 | 2.6   | 65.1 |
| 5. Middling machine-discharge          | 13.9 | 58.2 | ----- | 30.2 |

#### SAND FLOTATION FROM MIDDLE

|                                            |      |      |       |      |
|--------------------------------------------|------|------|-------|------|
| 6. Silicious froth-product to waste        | 3.9  | 12.5 | ----- | 1.8  |
| 7. Machine-discharge phosphate concentrate | 10.0 | 76.0 | 3.9   | 28.4 |

#### OVERALL RESULTS

|                                          |      |      |       |      |
|------------------------------------------|------|------|-------|------|
| 8. Total phosphate concentrate (4 and 7) | 32.6 | 76.8 | 3.0   | 93.5 |
| 9. Total tailing (3 and 6)               | 67.4 | 2.6  | ----- | 6.5  |

Thus, from ore containing 26.8% B. P. L. was obtained a phosphate concentrate containing 76.8% B. P. L. and only 3.0% insoluble, with a recovery of 93.5% of the B. P. L. in the ore; these results being achieved by the use of abnormally small quantities of reagents in the last step of the method.

#### Example II

This example illustrates the use of neutral flotation-water and agitative scrubbing of the rougher concentrate in the second step of the method.

A -35 mesh deslimed phosphate ore feed was conditioned in an aqueous pulp in the same manner and with the same quantities of negative-ion reagents, caustic soda and fuel oil and tall oil, as described in Example I, after which a rougher phosphate concentrate was removed as a flotation froth-product, leaving a silicious machine-discharge which was sent to waste.

The rougher phosphate concentrate was then subjected (in the second step) to an agitative scrubbing action in a paddle-type agitator for 3 minutes at approximately 50% solids with neutral tap water and then repulped in the flotation machine with neutral tap water at about 10% solids. The agitated rougher concentrate was then aerated and refloated in neutral tap water (without the addition of any pH modifying agents) thereby resulting in a retarded cleaner flotation which produced a high-grade phosphate concentrate containing a low sand content, and a middling machine-discharge consisting of both phosphate and sand particles.

The said middling was then agitated for about 3 minutes at approximately 50% solids with only 0.37 pound of  $H_2SO_4$  and was then washed and rinsed free of acid and spent negative-ion reagents. The thus-treated middling was repulped in a flotation machine at about 10% solids, conditioned for 15 seconds with positive-ion reagents consisting of only 0.03 pound of "Armac T" (tallow amine acetate), 0.14 pound of kerosene and 0.03 pound of pine oil frother (all in pounds per ton of original feed), then aerated and a silicious froth-product was removed and sent to waste, leaving a high-grade phosphate concentrate in the machine-discharge. The metallurgical results of this test are recorded in the following table:

#### ROUGHER PHOSPHATE FLOTATION

| Products                                | Percent weight | Percent B. P. L. | Percent insol. | Percent B. P. L. recovery |
|-----------------------------------------|----------------|------------------|----------------|---------------------------|
| 1. Feed                                 | 100.0          | 26.5             |                | 100.0                     |
| 2. Rougher concentrate froth-product    | 36.0           | 69.3             |                | 94.2                      |
| 3. Silicious machine-discharge to waste | 64.0           | 2.4              |                | 5.8                       |

#### RETARDED CLEANER FLOTATION

|                                        |      |      |     |      |
|----------------------------------------|------|------|-----|------|
| 4. Phosphate concentrate froth-product | 29.6 | 76.5 | 3.3 | 85.5 |
| 5. Middling machine-discharge          | 6.4  | 36.1 |     | 8.7  |

#### SAND FLOTATION FROM MIDDLEING

|                                            |     |      |     |     |
|--------------------------------------------|-----|------|-----|-----|
| 6. Silicious froth-product to waste        | 3.9 | 10.3 |     | 1.5 |
| 7. Machine-discharge phosphate concentrate | 2.5 | 76.5 | 3.0 | 7.2 |

#### OVERALL RESULTS

|                                          |      |      |     |      |
|------------------------------------------|------|------|-----|------|
| 8. Total phosphate concentrate (4 and 7) | 32.1 | 76.5 | 3.3 | 92.7 |
| 9. Total tailing (3 and 6)               | 67.9 | 2.9  |     | 7.3  |

The excellent over-all results of this example, as to both grade and recovery, and the economy in the amounts of acid and positive-ion reagents employed, in comparison with the amounts of those reagents employed in practicing the method of the Crago patent, are obvious.

#### Example III

This example illustrates the practicing of the

method by keeping the pulp level in the cleaner flotation cells well below the froth lip and paddling off only the top part of the froth, in the second step of the method.

A -35 mesh deslimed phosphate ore feed was conditioned with negative-ion reagents in an aqueous pulp, diluted, and a rougher phosphate concentrate was removed as a flotation froth-product in the manner described in Examples 1 and 2, except that the negative-ion reagent quantities used were 0.35 pound of caustic soda, 2.20 pounds of fuel oil and 0.21 pound of tall oil, all in pounds per ton of dry feed.

In the second step, the rougher phosphate concentrate was then repulped in the flotation cell with tap water at about 10% solids and subjected to retarded flotation which was achieved by holding the pulp level well below the froth lip of the cell and paddling off only the top part of the froth for a period of only 15 seconds (about one-third of the complete normal flotation time), thus producing a phosphate concentrate containing a minimum sand content and a middling machine-discharge consisting of both phosphate and sand particles.

The said middling was agitated for 3 minutes at approximately 50% solids with 1 pound of  $H_2SO_4$  and then washed and rinsed free of acid and spent negative-ion reagents. The deoiled and rinsed middling was repulped in the flotation machine at about 10% solids, conditioned for 15 seconds with only 0.06 pound of "Armac T" (tallow amine acetate), 0.2 pound of kerosene, and 0.06 pound of pine oil (all in pounds per ton of original feed), then aerated and a low-grade silicious froth-product was removed and sent to waste, leaving a high-grade phosphate concentrate in the machine-discharge which was combined with the phosphate concentrate produced in the second step. The metallurgical results of this test are recorded in the following table:

#### ROUGHER PHOSPHATE FLOTATION

| Products                                | Percent weight | Percent B. P. L. | Percent insol. | Percent B. P. L. recovery |
|-----------------------------------------|----------------|------------------|----------------|---------------------------|
| 1. Feed                                 | 100.0          | 27.2             |                | 100.0                     |
| 2. Rougher concentrate froth-product    | 34.1           | 74.4             |                | 93.2                      |
| 3. Silicious machine-discharge to waste | 65.9           | 2.8              |                | 6.8                       |

#### RETARDED CLEANER FLOTATION

|                                        |      |      |     |      |
|----------------------------------------|------|------|-----|------|
| 4. Phosphate concentrate froth-product | 22.7 | 76.7 | 3.1 | 64.0 |
| 5. Middling machine-discharge          | 11.4 | 69.8 |     | 20.2 |

#### SAND FLOTATION FROM MIDDLEING

|                                            |     |      |     |      |
|--------------------------------------------|-----|------|-----|------|
| 6. Silicious froth-product to waste        | 1.5 | 16.2 |     | 0.9  |
| 7. Machine-discharge phosphate concentrate | 9.9 | 78.0 | 1.9 | 28.3 |

#### OVERALL RESULTS

|                                          |      |      |     |      |
|------------------------------------------|------|------|-----|------|
| 8. Total phosphate concentrate (4 and 7) | 32.6 | 77.1 | 2.7 | 92.3 |
| 9. Total tailing (3 and 6)               | 67.4 | 3.1  |     | 7.7  |

These excellent over-all results as to both grade and recovery show that the process can be satisfactorily practiced, with a considerable reduction in the negative-ion reagents used in the rougher flotation (first step), by using mechani-

cal impediments to the flotation of the phosphate concentrate in the second step, by maintaining low flotation-cell pulp-levels, and by incomplete removal of the froth-product. Furthermore, this example illustrates the achieving of economy in the amounts of acid and positive-ion reagents employed in steps three and four, as compared with the far greater amounts of these reagents used in tests 4 and 5 of the Crago patent.

Various combinations of the procedures described for achieving retarded-flotation of phosphate in the second step have proved equally effective in producing a high-grade phosphate concentrate containing only a very small amount of sand; and a rich middling which was easily freed of negative-ion reagents, after which the sand was floated with a minimum of cationic collector reagent. For example, the procedures tried successfully have included agitation of the rougher concentrate (produced in the first step) followed by flotation in acid water, agitation with small amounts of acid followed by retarded-flotation in tap water. In general, the use of acid reduces the agitation required to produce the same retarded-flotation effect. Tests in which the rougher phosphate concentrates were subjected to agitative scrubbing for various lengths of time have shown that the retarded-flotation effect is proportional to the time of the agitation of the rougher concentrates. In general, the grade of the phosphate concentrate produced by retarded-flotation increases with the retarding effect, as does also the weight of the middling produced in the second step.

It seems to be a fact that the middlings (produced in the second step) appear to have flotation properties different from those of normal middlings. The usual middling from a normal phosphate cleaner flotation can be recirculated to the feed continuously with only a moderate build-up in the circuit until a stable condition is established. However, the middling produced by retarded flotation treatment of the rougher concentrate which has been tested by recirculation to the feed, continued to build up indefinitely and did not show any tendency to reach an equilibrium.

Various mineral acids, mineral acid salts, and organic acids have been used in the flotation water to retard the flotation of the phosphate concentrate and produce the middling, in the second step. These have included, for example, nitric acid, hydrochloric acid, propionic acid, potassium bisulfate, hydrofluosilicic acid, acetic acid and stannic chloride, producing waters varying from 3.0 pH to 5.7 pH. In general, the retarding effect on the flotation increases with the acidity of the flotation water.

The method of the present invention has been successfully tested with the use of a number of negative-ion collector reagents to produce the rougher phosphate concentrate which is then subjected to a retarded-flotation in the manner described. The negative-ion collector reagents tested include red oil (crude oleic acid), fish oil fatty acids, tall oil and tall oil soap, and the petroleum sulfonate commonly known as mahogany sulfonate.

The flotation of silicious gangue from the acid-treated and rinsed middling (in the fourth step) has been carried out with different positive-ion collector reagents, such as, for example, "Armac T" (Armour & Company's tallow amine acetate), technical lauryl amine hydrochloride, and a

7 "Rosin Amine D Acetate" (a Hercules Company product).

It is a peculiar fact that the positive-ion reagent requirement for floating the silicious gangue from the acid-treated and rinsed middling is only a fraction of that required to float the same amount of silicious gangue from the acid-treated rougher concentrate in the process of the Crago patent. Obviously, to produce the same high-grade total concentrate the two processes must remove the same amount of silicious gangue from the rougher phosphate concentrate. Comparison tests have shown that the amine reagent requirement for floating this silicious gangue from the acid-treated and rinsed middling according to the present method, is only one-half, one-third or less of that required to float the same silicious gangue from the total acid-treated rougher concentrate according to the process of the Crago patent. It appears that in the present method the lesser amount of phosphate present in the middling produced by retarded-flotation treatment allows a decrease in the amount of positive-ion reagent required.

The improvement in the percentage recovery of phosphate achieved by the present invention, over the method of the Crago patent, is shown by comparison of the tests in the Crago patent and the examples in the present specification. In Crago's tests 4 and 5, the recoveries are 79.2% and 87.5% respectively (see the tabulation on page 3 of the Crago patent). In the examples hereinbefore given, the over-all recoveries are 93.5%, 92.7% and 92.3% respectively. Since the amount of phosphatic material treated in the Florida phosphate area alone runs into millions of tons annually, this improvement in over-all recovery is important.

40 The economy in the amount of positive-ion reagents resulting from the applicants' method, in comparison with the method of the Crago patent, is also important. In tests 4 and 5 reported on page 3 of the Crago patent, 0.20 lb. of octadecylamine acetate were required. Whereas, in Examples 1, 2 and 3 of the applicant's specification only .025 lb., .03 lb. and .06 lb. of amine acetate were used. Thus, it is apparent that the applicants' method permits the use of very considerably less positive-ion reagents than is required in the Crago method. Since positive-ion reagents are rather expensive, economy in the use of them is important.

Obviously, therefore, the applicants' method is a valuable improvement on the method of the Crago patent.

55 What is claimed is:

1. A method of concentrating phosphate minerals from their ores which comprises the following sequence of steps: (1) subjecting the ore in an aqueous pulp to a froth-flotation treatment with negative-ion reagents, thereby producing a froth-product which is a rougher concentrate of the phosphate values mixed with some silicious gangue; (2) subjecting said rougher concentrate in an aqueous pulp to retarded froth-flotation treatment and removing as a part of the final product a froth-product having a low insoluble content, and a middling residue; (3) subjecting said middling in an aqueous pulp to treatment with a mineral acid followed by rinsing with water, thereby removing from said middling substantially all of said negative-ion reagents; and (4) subjecting said acid-treated and rinsed middling in an aqueous pulp to a froth-flotation treatment with positive-ion reagents thereby pro-

ducing a froth-product mostly composed of siliceous gangue which is discarded, and a residue which is a high-grade phosphate concentrate and can be combined with the previously mentioned commercial-grade phosphate concentrate; thereby producing a final high-grade phosphate concentrate containing a high proportion of the phosphate in the ore.

2. The method of concentrating phosphate minerals according to claim 1, using a weakly-acid flotation water in the retarded froth-flotation treatment in the second step (2).

3. The method of concentrating phosphate minerals according to claim 1, using neutral flotation water and agitative scrubbing of the rougher phosphate concentrate in a thick pulp as a part of the retarded froth-flotation treatment in the second step (2).

4. The method of concentrating phosphate minerals according to claim 1, in which in the 20

retarded froth-flotation treatment in the second step (2) only the top of the froth-product is removed.

JAMES B. DUKE.  
WESLEY M. HOUSTON.

References Cited in the file of this patent

UNITED STATES PATENTS

| Number    | Name            | Date          |
|-----------|-----------------|---------------|
| 1,480,884 | Dolbear         | Jan. 15, 1924 |
| 2,293,640 | Crago           | Aug. 18, 1842 |
| 2,350,943 | Thompson et al. | June 6, 1944  |
| 2,461,813 | Duke            | Feb. 15, 1949 |

OTHER REFERENCES

Milling Methods for 1934, published by the A. I. M. M. E., New York, New York, 1935, pages 452 and 460 (copy in Div. 25).

Taggart, Handbook of Mineral Dressing, © 1945, Section 12, page 100 (copy in Div. 25).